

# UNITED STATES PATENT OFFICE.

FOSTER MILLIKEN, OF LAWRENCE, NEW YORK, ASSIGNOR TO FOSTER MILLIKEN,  
S. FULLERTON WEAVER, AND JAMES M. REFFLER, AS TRUSTEES.

## ALLOY.

1,385,223.

Specification of Letters Patent. Patented July 19, 1921.

No Drawing.

Application filed May 24, 1920. Serial No. 383,888.

To all whom it may concern:

Be it known that I, FOSTER MILLIKEN, a citizen of the United States, and a resident of Lawrence, in the county of Nassau and State of New York, have invented a new and Improved Alloy, of which the following is a full, clear, and exact description.

The invention relates to alloys containing aluminum and lead as the principal ingredients, and its object is to provide a new and improved alloy of this type characterized by pronounced density and ability to withstand pressure.

Another object is to provide an alloy particularly suited to resist nitric acids, nitrate derivatives, ammonia, picric acid and other similar acids having deleterious influences when subjecting ordinary aluminum alloys to the action thereof.

The alloy consists of the following ingredients in about the proportions stated, namely:

Aluminum----- 89 to 94 per cent.  
Lead ----- 5 to 10 " "  
25 and a trace of an oxidizing material such as metallic magnesium.

In practice, the aluminum and the lead are mixed while in a molten state and about 1

to 2 per cent. of metallic magnesium is 30 added to deoxidize or purify both the aluminum and the lead with a trace of the oxidizing material being incorporated in the alloy and the remainder passing away with the slag.

It is understood that aluminum alloys as now generally formed are porous and one of the properties of my improved alloy as herein set forth is its increased density owing to the use of the purified lead and the 40 purified aluminum.

Having thus described my invention, I claim as new and desire to secure by Letters Patent:—

An alloy containing aluminum, lead, and 45 an oxidizing agent, the aluminum and the lead being in a purified state and in proportion substantially as specified, the said oxidizing agent being a portion of 1 to 2 per cent. of the deoxidizing agent used as the 50 medium for purifying the said aluminum and the said lead and remaining as an integral part of the alloy after purification of the said aluminum and lead, the said alloy being characterized by increased density, 55 ability to withstand pressure and high resistance to corrosion.

FOSTER MILLIKEN.